



US008092972B2

(12) **United States Patent**  
**Zhou et al.**

(10) **Patent No.:** **US 8,092,972 B2**  
(45) **Date of Patent:** **Jan. 10, 2012**

(54) **TONER COMPOSITIONS**

(75) Inventors: **Ke Zhou**, Mississauga (CA); **Edward G. Zwarts**, Mississauga (CA); **Karen Ann Moffat**, Brantford (CA)

(73) Assignee: **Xerox Corporation**, Norwalk, CT (US)

(\*) Notice: Subject to any disclaimer, the term of this patent is extended or adjusted under 35 U.S.C. 154(b) by 689 days.

(21) Appl. No.: **12/198,981**

(22) Filed: **Aug. 27, 2008**

(65) **Prior Publication Data**

US 2010/0055592 A1 Mar. 4, 2010

(51) **Int. Cl.**

**G03G 5/00** (2006.01)

(52) **U.S. Cl.** ..... **430/137.14**; 430/137.11; 430/137.12; 430/108.1; 430/110.2

(58) **Field of Classification Search** ..... 430/137.11, 430/137.12, 137.13, 137.14, 108.1, 108.4, 430/108.8, 110.2

See application file for complete search history.

(56) **References Cited**

## U.S. PATENT DOCUMENTS

|             |         |                  |
|-------------|---------|------------------|
| 3,590,000 A | 6/1971  | Palermi et al.   |
| 3,800,588 A | 4/1974  | Larson et al.    |
| 3,847,604 A | 11/1974 | Hagenbach et al. |
| 4,295,990 A | 10/1981 | Verbeek et al.   |
| 4,298,672 A | 11/1981 | Lu               |
| 4,338,390 A | 7/1982  | Lu               |
| 4,935,326 A | 6/1990  | Creatura et al.  |
| 4,937,166 A | 6/1990  | Creatura et al.  |
| 5,236,629 A | 8/1993  | Mahabadi et al.  |

|              |         |                            |
|--------------|---------|----------------------------|
| 5,290,654 A  | 3/1994  | Sacripante et al.          |
| 5,302,486 A  | 4/1994  | Patel et al.               |
| 5,330,874 A  | 7/1994  | Mahabadi et al.            |
| 5,346,797 A  | 9/1994  | Kmiecik-Lawrynowicz et al. |
| 5,364,729 A  | 11/1994 | Kmiecik-Lawrynowicz et al. |
| 5,403,693 A  | 4/1995  | Patel et al.               |
| 5,418,108 A  | 5/1995  | Kmiecik-Lawrynowicz et al. |
| 5,501,935 A  | 3/1996  | Patel et al.               |
| 5,527,658 A  | 6/1996  | Hopper et al.              |
| 5,585,215 A  | 12/1996 | Ong et al.                 |
| 5,650,255 A  | 7/1997  | Ng et al.                  |
| 5,650,256 A  | 7/1997  | Veregin et al.             |
| 5,773,185 A  | 6/1998  | Yachi et al.               |
| 5,853,943 A  | 12/1998 | Cheng et al.               |
| 6,063,827 A  | 5/2000  | Sacripante et al.          |
| 6,214,507 B1 | 4/2001  | Sokol et al.               |
| 6,395,442 B1 | 5/2002  | Hayashi et al.             |

(Continued)

## FOREIGN PATENT DOCUMENTS

JP 2007 086211 4/2007

(Continued)

## OTHER PUBLICATIONS

European Search Report for European Patent No. EP 09 16 7759 dated Jan. 5, 2010.

Primary Examiner — Mark F Huff

Assistant Examiner — Stewart Fraser

(74) Attorney, Agent, or Firm — MDIP LLC

(57) **ABSTRACT**

Toner particles are provided which may, in embodiments, include a core and a shell formed in situ. The resins utilized to form the core, the shell, or both, may be contacted with a water soluble initiator. The resin, in embodiments present in the shell, cross-links at a temperature near the temperature for coalescence, and may prevent a crystalline resin in the core from migrating to the toner surface.

13 Claims, 1 Drawing Sheet



**U.S. PATENT DOCUMENTS**

|              |     |         |                               |              |     |         |                            |
|--------------|-----|---------|-------------------------------|--------------|-----|---------|----------------------------|
| 6,593,049    | B1  | 7/2003  | Veregin et al.                | 2007/0037086 | A1  | 2/2007  | Skorokhod et al.           |
| 6,756,176    | B2  | 6/2004  | Stegamat et al.               | 2007/0092821 | A1  | 4/2007  | Sato et al.                |
| 6,830,860    | B2  | 12/2004 | Sacripante et al.             | 2007/0141500 | A1  | 6/2007  | Sugimoto et al.            |
| 7,214,463    | B2  | 5/2007  | Patel et al.                  | 2007/0207400 | A1  | 9/2007  | Ahuja et al.               |
| 7,307,111    | B2  | 12/2007 | Moffat et al.                 | 2007/0254229 | A1  | 11/2007 | Patel et al.               |
| 2005/0287461 | A1  | 12/2005 | Sweeney et al.                | 2008/0090163 | A1* | 4/2008  | Agur et al. .... 430/108.1 |
| 2006/0216625 | A1* | 9/2006  | Maehata et al. .... 430/109.3 | 2008/0096119 | A1  | 4/2008  | Yamamoto et al.            |
| 2006/0222991 | A1  | 10/2006 | Sacripante et al.             |              |     |         |                            |
| 2006/0269858 | A1  | 11/2006 | McDougall et al.              |              |     |         |                            |
| 2006/0292477 | A1  | 12/2006 | Daimon et al.                 |              |     |         |                            |
| 2007/0003856 | A1  | 1/2007  | Farrugia et al.               |              |     |         |                            |

**FOREIGN PATENT DOCUMENTS**

JP 2008 070755 3/2008

\* cited by examiner

**FIG. 1****FIG. 2**

# 1

## TONER COMPOSITIONS

### CROSS-REFERENCE TO RELATED APPLICATIONS

This application is related to co-pending U.S. application Ser. Nos. 12/198,999 and 12/199,115, both filed on Aug. 27, 2008, the entire disclosures of each of which are hereby incorporated by reference in their entirety.

### BACKGROUND

The present disclosure relates to toners suitable for electrophotographic apparatuses.

Numerous processes are within the purview of those skilled in the art for the preparation of toners. Emulsion aggregation (EA) is one such method. These toners may be formed by aggregating a colorant with a latex polymer formed by emulsion polymerization. For example, U.S. Pat. No. 5,853,943, the disclosure of which is hereby incorporated by reference in its entirety, is directed to a semi-continuous emulsion polymerization process for preparing a latex by first forming a seed polymer. Other examples of emulsion/aggregation/coalescing processes for the preparation of toners are illustrated in U.S. Pat. Nos. 5,403,693, 5,418,108, 5,364,729, and 5,346,797, the disclosures of each of which are hereby incorporated by reference in their entirety. Other processes are disclosed in U.S. Pat. Nos. 5,527,658, 5,585,215, 5,650,255, 5,650,256 and 5,501,935, the disclosures of each of which are hereby incorporated by reference in their entirety.

Polyester EA ultra low melt (ULM) toners have been prepared utilizing amorphous and crystalline polyester resins. While these toners may exhibit excellent fusing properties including crease minimum fixing temperature (MFT) and fusing latitude, peak gloss of these toners may be unacceptably high. Improved toners thus remain desirable.

### SUMMARY

The present disclosure provides particles suitable for use in toners and methods for their production. In embodiments, a process of the present disclosure may include contacting at least one amorphous resin with at least one crystalline resin in an aqueous emulsion to form small particles, wherein the emulsion includes an optional colorant, an optional surfactant, and an optional wax; aggregating the small particles to form a plurality of larger aggregates; contacting the larger aggregates with an emulsion including the at least one amorphous resin or a different at least one amorphous resin, or both, to form a resin coating over the larger aggregates; coalescing the larger aggregates within the resin coating and simultaneously or subsequently crosslinking either the larger aggregates or the resin coating or both, to form a plurality of crosslinked particles including a core and a shell; adding an at least one water soluble initiator at any stage in the process prior to the formation of the crosslinked particles; and recovering the crosslinked particles.

In embodiments, a process of the present disclosure may include contacting at least one amorphous resin with at least one crystalline resin in an aqueous emulsion optionally in combination with at least one water soluble initiator such as potassium persulfate, ammonium persulfate, sodium persulfate, 2,2'-azobis[2-(2-imidazolin-2-yl)propane]dihydrochloride, 2,2'-azobis[2-(2-imidazolin-2-yl)propane]disulfate dehydrate, 2,2'-azobis(2-methylpropionamidine)dihydrochloride, 2,2'-azobis[N-(2-carboxyethyl)-2-methylpropionamidine]hydrate, 2,2'-azobis{2-[1-(2-hydroxyethyl)-2-imidazolin-2-yl]propane}dihydrochloride, 2,2'-azobis[2-(2-imidazolin-2-yl)propane]disulfate dehydrate, 2,2'-azobis(2-methylpropionamidine)dihydrochloride, 2,2'-azobis{2-[1-(2-hydroxyethyl)-2-imidazolin-2-yl]propane}dihydrochloride, 2,2'-azobis(1-imino-1-pyrrolidino-2-ethylpropane)dihydrochloride, 2,2'-azobis{2-methyl-N-[1,1-bis(hydroxymethyl)-2-hydroxyethyl]propionamide}, 2,2'-azobis{2-methyl-N-(2-hydroxyethyl)propionamide}, and combinations thereof to form a crosslinked resin: contacting the aqueous emulsion with an optional colorant, at least one surfactant, and an optional wax to form small particles; aggregating the small particles to form a plurality of larger aggregates; contacting the larger aggregates with an emulsion including at least one amorphous resin optionally in combination with at least one water soluble initiator such as potassium persulfate, ammonium persulfate, sodium persulfate, 2,2'-azobis[2-(2-imidazolin-2-yl)propane]dihydrochloride, 2,2'-azobis[2-(2-imidazolin-2-yl)propane]disulfate dehydrate, 2,2'-azobis(2-methylpropionamidine)dihydrochloride, 2,2'-azobis{2-[1-(2-hydroxyethyl)-2-imidazolin-2-yl]propane}dihydrochloride, 2,2'-azobis(1-imino-1-pyrrolidino-2-ethylpropane)dihydrochloride, 2,2'-azobis{2-methyl-N-[1,1-bis(hydroxymethyl)-2-hydroxyethyl]propionamide}, 2,2'-azobis{2-methyl-N-(2-hydroxyethyl)propionamide}, and combinations thereof to form a crosslinked resin coating over the larger aggregates; coalescing the larger aggregates possessing the resin coating to form toner particles; heating the toner particles to a temperature of from about 70° C. to about 100° C. to crosslink the amorphous resin; and recovering the toner particles.

5 zolin-2-yl]propane}dihydrochloride, 2,2'-azobis[2-(2-imidazolin-2-yl)propane], 2,2'-azobis(1-imino-1-pyrrolidino-2-ethylpropane)dihydrochloride, 2,2'-azobis{2-methyl-N-[1,1-bis(hydroxymethyl)-2-hydroxyethyl]propionamide}, 2,2'-azobis[2-methyl-N-(2-hydroxyethyl)propionamide], 2,2'-azobis{2-[1-(2-hydroxyethyl)-2-imidazolin-2-yl]propane}dihydrochloride, 2,2'-azobis(1-imino-1-pyrrolidino-2-ethylpropane)dihydrochloride, 2,2'-azobis{2-methyl-N-[1,1-bis(hydroxymethyl)-2-hydroxyethyl]propionamide}, 2,2'-azobis{2-methyl-N-(2-hydroxyethyl)propionamide}, and combinations thereof to form a crosslinked resin: contacting the aqueous emulsion with an optional colorant, at least one surfactant, and an optional wax to form small particles; aggregating the small particles to form a plurality of larger aggregates; contacting the larger aggregates with an emulsion including at least one amorphous resin optionally in combination with at least one water soluble initiator such as potassium persulfate, ammonium persulfate, sodium persulfate, 2,2'-azobis[2-(2-imidazolin-2-yl)propane]dihydrochloride, 2,2'-azobis[2-(2-imidazolin-2-yl)propane]disulfate dehydrate, 2,2'-azobis(2-methylpropionamidine)dihydrochloride, 2,2'-azobis{2-[1-(2-hydroxyethyl)-2-imidazolin-2-yl]propane}dihydrochloride, 2,2'-azobis(1-imino-1-pyrrolidino-2-ethylpropane)dihydrochloride, 2,2'-azobis{2-methyl-N-[1,1-bis(hydroxymethyl)-2-hydroxyethyl]propionamide}, 2,2'-azobis{2-methyl-N-(2-hydroxyethyl)propionamide}, and combinations thereof to form a crosslinked resin coating over the larger aggregates; coalescing the larger aggregates possessing the resin coating to form toner particles; heating the toner particles to a temperature of from about 70° C. to about 100° C. to crosslink the amorphous resin; and recovering the toner particles.

10 15 20 25 30 35 40 45 50 55 60 65

In embodiments, a toner of the present disclosure may include particles including a core including at least one amorphous resin, at least one crystalline resin, and one or more optional ingredients selected from the group consisting of colorants, waxes, reaction products of water soluble initiators with the amorphous resin, and combinations thereof, and a shell including at least one amorphous resin crosslinked with at least one water soluble initiator.

### BRIEF DESCRIPTION OF THE DRAWINGS

Various embodiments of the present disclosure will be described herein below with reference to the figure wherein:

FIG. 1 is a graph comparing the rheological properties of a toner produced in accordance with the present disclosure compared with a control toner; and

FIG. 2 is a graph depicting the gloss properties of toners of the present disclosure.

### DETAILED DESCRIPTION

The present disclosure provides toner particles having desirable gloss properties. The toner particles possess a core-shell configuration, with a polyester gel or partially crosslinked polyester in the core, the shell, or both. In embodiments, the gloss of the resulting toner may be reduced by cross-linking the polyester in the core and/or shell with a water soluble initiator during toner preparation.

#### Core Resins

Any resin may be utilized in forming a toner core of the present disclosure. In the event that the core resin is to be crosslinked, any crosslinkable resin may be utilized. Such resins, in turn, may be made of any suitable monomer. Suitable monomers useful in forming the resin include, but are not limited to, styrenes, acrylates, methacrylates, butadienes, isoprenes, acrylic acids, methacrylic acids, acrylonitriles, diol, diacid, diamine, diester, mixtures thereof: and the like. Any

monomer employed may be selected depending upon the particular polymer to be utilized.

In embodiments, the core resins may be an amorphous resin, a crystalline resin, and a combination. In further embodiments, the polymer utilized to form the resin core may be a polyester resin, including the resins described in U.S. Pat. Nos. 6,593,049 and 6,756,176, the disclosures of each of which are hereby incorporated by reference in their entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, the resin may be a polyester resin formed by reacting a diol with a diacid in the presence of an optional catalyst. For forming a crystalline polyester, suitable organic diols include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,12-dodecanediol and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol may be, for example, selected in an amount of from about 40 to about 60 mole percent, in embodiments from about 42 to about 55 mole percent, in embodiments from about 45 to about 53 mole percent, and the alkali sulfo-aliphatic diol can be selected in an amount of from about 0 to about 10 mole percent, in embodiments from about 1 to about 4 mole percent of the resin.

Examples of organic diacids or diesters including vinyl diacids or vinyl diesters selected for the preparation of the crystalline resins include oxalic acid, succinic acid, glutaric acid, adipic acid, suberic acid, azelaic acid, sebatic acid, fumaric acid, dimethyl fumarate, dimethyl itaconate, cis, 1,4-diacetoxy-2-butene, diethyl fumarate, diethyl maleate, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof, and an alkali sulfo-organic diacid such as the sodio, lithio or potassium salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfo-phenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfoethanediol, 2-sulfopropanediol, 2-sulfobutanediol, 3-sulfopentanediol, 2-sulfohexanediol, 3-sulfo-2-methylpentanediol, 2-sulfo-3,3-dimethylpentanediol, sulfo-p-hydroxybenzoic acid, N,N-bis(2-hydroxyethyl)-2-amino ethane sultanate, or mixtures thereof. The organic diacid may be selected in an amount of, for example, in embodiments from about 40 to about 60 mole percent, in embodiments from about 42 to about 52 mole percent, in embodiments from about 45 to about 50 mole percent, and the alkali sulfo-aliphatic diacid can be selected in an amount of from about 1 to about 10 mole percent of the resin.

Examples of crystalline resins include polyesters, polyamides, polyimides, polyolefins, polyethylene, polybutylene, polyisobutyrate, ethylene-propylene copolymers, ethylene-vinyl acetate copolymers, polypropylene, mixtures thereof, and the like. Specific crystalline resins may be polyester based, such as poly(ethylene-adipate), poly(propylene-adipate), poly(butylene-adipate), poly(pentylene-adipate), poly-

The crystalline resin may be present, for example, in an amount of from about 5 to about 50 percent by weight of the toner components, in embodiments from about 5 to about 35 percent by weight of the toner components. The crystalline resin can possess various melting points of, for example, from about 30° C. to about 120° C. in embodiments from about 50° C. to about 90° C. The crystalline resin may have a number average molecular weight ( $M_n$ ), as measured by gel permeation chromatography (GPC) of, for example, from about 1,000 to about 50,000, in embodiments from about 2,000 to about 25,000, and a weight average molecular weight ( $M_w$ ) of, for example, from about 2,000 to about 100,000, in embodiments from about 3,000 to about 80,000, as determined by Gel Permeation Chromatography using polystyrene standards. The molecular weight distribution ( $M_w/M_n$ ) of the crystalline resin may be, for example, from about 2 to about 6, in embodiments from about 2 to about 4.

Examples of diacid or diesters including vinyl diacids or vinyl diesters selected for the preparation of amorphous polyesters include dicarboxylic acids or diesters such as terephthalic acid, phthalic acid, isophthalic acid, fumaric acid, dimethyl fumarate, dimethyl itaconate, cis, 1,4-diacetoxy-2-butene, diethyl fumarate, diethyl maleate, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 52 mole percent of the resin, in embodiments from about 45 to about 50 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanedimethanol, 1,3-cyclohexanedimethanol, xylenedimethanol, cyclohexanediol, diethylene glycol, bis(2-hydroxyethyl) oxide, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

Polycondensation catalysts which may be utilized for either the crystalline or amorphous polyesters include tetraalkyl titanates, dialkyltin oxides such as dibutyltin oxide, tetraalkyltins such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole percent to about 5 mole percent based on the starting diacid or diester used to generate the polyester resin.

In embodiments, suitable amorphous resins include polyesters, polyamides, polyimides, polyolefins, polyethylene, polybutylene, polyisobutylene, ethylene-propylene copolymers, ethylene-vinyl acetate copolymers, polypropylene, combinations thereof, and the like. Examples of amorphous resins which may be utilized include poly(styrene-acrylate) resins, crosslinked, for example, from about 10 percent to about 70 percent, poly(styrene-acrylate) resins, poly(styrene-methacrylate) resins, crosslinked poly(styrene-methacrylate) resins, poly(styrene-butadiene) resins, crosslinked poly(styrene-butadiene) resins, alkali sulfonated-polyester resins, branched alkali sulfonated-polyester resins, alkali sulfonated-polyimide resins, branched alkali sulfonated-polyimide resins, alkali sulfonated poly(styrene-acrylate) resins, crosslinked alkali sulfonated poly(styrene-acrylate) resins, poly(styrene-methacrylate) resins, crosslinked alkali sulfonated-poly(styrene-methacrylate) resins, alkali sulfonated-poly(styrene-butadiene) resins, and crosslinked alkali sul-

fonated poly(styrene-butadiene) resins. Alkali sulfonated polyester resins may be useful in embodiments, such as the metal or alkali salts of copoly(ethylene-terephthalate)-copol (ethylene-5-sulfo-isophthalate), copoly(propylene-terephthalate)-copol (propylene-5-sulfo-isophthalate), copoly(diethylene-terephthalate)-copol (diethylene-5-sulfo-isophthalate), copoly(propylene-diethylene-terephthalate)-copol (propylene-diethylene-5-sulfoisophthalate), copoly(propylene-butylene-terephthalate)-copol (propylene-butylene-5-sulfo-isophthalate), copoly(propoxylated bisphenol-A-fumarate)-copol (propoxylated bisphenol A-5-sulfo-isophthalate), copoly(ethoxylated bisphenol-A-fumarate)-copol (ethoxylated bisphenol A-5-sulfo-isophthalate), and copoly(ethoxylated bisphenol-A-5-sulfo-isophthalate), and wherein the alkali metal is, for example, a sodium, lithium or potassium ion.

Examples of other suitable resins or polymers which may be utilized include, but are not limited to, poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), and poly(styrene-butyl acrylate-acrylonitrile-acrylic acid), and combinations thereof. The polymer may be block, random, or alternating copolymers.

In embodiments, the core resin is a crosslinkable resin. A crosslinkable resin is a resin comprising crosslinkable group or groups such as  $C=C$  bond. The resin can be crosslinked for example through a free radical polymerization with an initiator. In embodiments, an unsaturated polyester resin may be utilized as a latex resin. Examples of such resins include those disclosed in U.S. Pat. No. 6,063,827, the disclosure of which is hereby incorporated by reference in its entirety. Exemplary unsaturated polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate) and combinations thereof.

In embodiments, a suitable polyester resin may be an amorphous polyester such as a poly(propoxylated bisphenol A co-fumarate) resin having the following formula (I):



wherein m may be from about 5 to about 1000.

An example of a linear propoxylated bisphenol A fumarate resin which may be utilized as a latex resin is available under the trade name SPARII from Resana S/A Industrias Quimicas, Sao Paulo Brazil. Other propoxylated bisphenol A fumarate resins that may be utilized and are commercially available include GTUF and FPESL-2 from Kao Corporation, Japan, and EM181635 from Reichhold, Research Triangle Park, N.C. and the like.

Suitable crystalline resins include those disclosed in U.S. Patent Application Publication No. 2006/0222991, the disclosure of which is hereby incorporated by reference in its entirety. In embodiments, a suitable crystalline resin may include a resin composed of ethylene glycol and a mixture of dodecanedioic acid and fumaric acid co-monomers with the following formula:



wherein b is from 5 to 2000 and d is from 5 to 2000.

For example, in embodiments, a poly(propoxylated bisphenol A co-fumarate) resin of formula I as described above may be combined with a crystalline resin of formula II to form a core.

In embodiments, as noted above, a core resin may be partially crosslinked in situ during formation toner particles to form a "partially crosslinked polyester resin" or a "polyester gel".

In order to partially crosslink the polyester and form a polyester gel, in embodiments it may be desirable to add a water soluble initiator to the resin utilized to form the core to enhance crosslinking and the resulting formation of the polyester gel. Suitable water soluble initiators which may be utilized to crosslink the resin in the core include, but are not limited to, persulfates, including potassium persulfate, ammonium persulfate, sodium persulfate, water soluble azo initiator including 2,2'-azobis[2-(2-imidazolin-2-yl)propane] dihydrochloride, 2,2'-azobis[2-(2-imidazolin-2-yl)propane] disulfate dehydrate, 2,2'-azobis(2-methylpropionamidine)dihydrochloride, 2,2'-azobis[N-(2-carboxyethyl)-2-methylpropionamidine]hydrate, 2,2'-azobis{2-[1-(2-hydroxyethyl)-2-imidazolin-2-yl]propane} dihydrochloride, 2,2'-azobis[2-(2-imidazolin-2-yl)propane], 2,2'-azobis(1-imino-1-pyrrolidino-2-ethylpropoxide)dihydrochloride, 2,2'-azobis{2-methyl-N-[1,1-bis(hydroxymethyl)-2-hydroxyethyl]propionamide}, 2,2'-azobis[2-methyl-N-(2-hydroxyethyl)propionamide], combinations thereof, and the like.

In embodiments, water soluble initiators may be dissolved in water or a similar solvent and added to the resin.

The partial crosslinking of the resin utilized to form the core may occur while heating to a temperature of from about 25° C. to about 99° C., in embodiments from about 40° C. to about 90° C. Partial crosslinking forming the core may take place for a period of time of from about 1 minute to about 10 hours, in embodiments from about 5 minutes to about 5 hours.

The amount of initiator utilized to crosslink the polyester may be from about 0.05 percent by weight to about 20 percent by weight of the resin utilized to form the core, in embodiments from about 0.1 percent by weight to about 10 percent by weight, or from about 0.5 percent by weight to about 5 percent by weight of the resin utilized to form the core.

In embodiments, the amorphous resin or combination of amorphous resins utilized in the core may have a glass transition temperature of from about 30° C. to about 80° C., in embodiments from about 35° C. to about 70° C. In further embodiments, the combined resins utilized in the core may have a melt viscosity of from about 10 to about 1,000,000 Pa\*S at about 130° C., in embodiments from about 20 to about 100,000 Pa\*S.

One, two, or more toner resins may be used. In embodiments where two or more toner resins are used, the toner resins may be in any suitable ratio (e.g., weight ratio) such as for instance about 10% (first resin)/90% (second resin) to about 90% (first resin)/10% (second resin).

In embodiments, the resin may be formed by condensation polymerization methods.

The resin described above may be utilized to form toner compositions. Such toner compositions may include optional colorants, waxes, and other additives. Toners may be formed utilizing any method within the purview of those skilled in the art.

#### Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl

ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, available from Rhone-Poulenac as IGEPAL CA-210<sup>TM</sup>, IGEPAL CA-520<sup>TM</sup>, IGEPAL CA-720<sup>TM</sup>, IGEPAL CO-890<sup>TM</sup>, IGEPAL CO-720<sup>TM</sup>, IGEPAL CO-290<sup>TM</sup>, IGEPAL CA-210<sup>TM</sup>, ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNERONIC PE/F, in embodiments SYNPONIC PE/F 108.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, acids such as abitic acid available from Aldrich, NEOGEN R<sup>TM</sup>, NEOGEN SC<sup>TM</sup> obtained from Daiichi Kogyo Seiyaku, combinations thereof, and the like. Other suitable anionic surfactants include, in embodiments, DOWFAX<sup>TM</sup> 2A 1, an alkylidiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL<sup>TM</sup> and ALKAQUATT<sup>TM</sup>, available from Alkaril Chemical Company. SANIZOL<sup>TM</sup> (benzalkonium chloride), available from Kao Chemicals, and the like, and mixtures thereof.

#### Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 0.1 to about 35 percent by weight of the toner, or from about 1 to about 15 weight percent of the toner, or from about 3 to about 10 percent by weight of the toner.

As examples of suitable colorants, mention may be made of carbon black like REGAL330<sup>®</sup>; magnetites, such as Mobay magnetites MO8029<sup>TM</sup>, MO8060<sup>TM</sup>; Columbian magnetites; MAPICO BLACK<sup>TM</sup> and surface treated magnetites; Pfizer magnetites CB4799<sup>TM</sup>, CB5300<sup>TM</sup>, CB5600<sup>TM</sup>, MCX6369<sup>TM</sup>; Bayer magnetites, BAYFERROX8600<sup>TM</sup>, 8610<sup>TM</sup>; Northern Pigments magnetites, NP-604<sup>TM</sup>, NP-608<sup>TM</sup>; Magnox magnetites TMB-100<sup>TM</sup>, or TMB-104<sup>TM</sup>; and the like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals. HELIOGEN BLUE L6900<sup>TM</sup>, D6840<sup>TM</sup>, D7080<sup>TM</sup>, D7020<sup>TM</sup>, PYLAM OIL BLUE<sup>TM</sup>, PYLAM OIL YELLOW<sup>TM</sup>, PIGMENT BLUE 1<sup>TM</sup>

available from Paul Uhlich & Company, Inc., PIGMENT VIOLET 1<sup>TM</sup>, PIGMENT RED 48<sup>TM</sup>, LEMON CHROME YELLOW DCC 1026<sup>TM</sup>, E. D. TOLUIDINE RED<sup>TM</sup> and BON RED C<sup>TM</sup> available from Dominion Color Corporation, Ltd., Toronto, Ontario, NOVAPERM YELLOW FGL<sup>TM</sup>, HOSTAPERM PINK E<sup>TM</sup> from Hoechst, and CINQUASIA MAGENTA<sup>TM</sup> available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyans include copper tetra(ocotadecyl sulfonamido) phthalocyanine, x-copper phthalocyanine pigment listed in the Color Index as CI 74160, CI Pigment Blue, Pigment Blue 15:3, and Anthrathrene Blue, identified in the Color Index as CI 69810, Special Blue X-2137, and the like. Illustrative examples of yellows are diarylide yellow 3,3-dichlorobenzidine acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK<sup>TM</sup>, and cyan components may also be selected as colorants. Other known colorants can be selected, such as Levanyl Black A-SF (Miles, Bayer) and Sunperse Carbon Black LHD 9303 (Sun Chemicals), and colored dyes such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E. D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing, and the like.

#### Wax

Optionally, a wax may also be combined with the resin and a colorant in forming toner particles. When included, the wax may be present in an amount of, for example, from about 1 weight percent to about 25 weight percent of the toner particles, in embodiments from about 5 weight percent to about 20 weight percent of the toner particles.

Waxes that may be selected include waxes having, for example, a weight average molecular weight of from about 500 to about 20,000, in embodiments from about 1,000 to about 10,000. Waxes that may be used include, for example, polyolefins such as polyethylene, polypropylene, and polybutene waxes such as commercially available from Allied

## 11

Chemical and Petrolite Corporation, for example POLY-WAX<sup>TM</sup> polyethylene waxes from Baker Petrolite, wax emulsions available from Michaelman, Inc. and the Daniels Products Company, EPOLENE N-15<sup>TM</sup> commercially available from Eastman Chemical Products, Inc., and VISCOL 550-P<sup>TM</sup>, a low weight average molecular weight polypropylene available from Sanyo Kasei K. K.; plant-based waxes, such as carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax, and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol multimers, such as diethyleneglycol monostearate, dipropylene-glycol distearate, diglyceryl distearate, and triglyceryl tetraestearate; sorbitan higher fatty acid ester waxes, such as sorbitan monostearate, and cholesterol higher fatty acid ester waxes, such as cholesteryl stearate. Examples of functionalized waxes that may be used include, for example, amines, amides, for example AQUA SUPERSLIP 6550<sup>TM</sup>, SUPER-SLIP 6530<sup>TM</sup> available from Micro Powder Inc., fluorinated waxes, for example POLYFLUO 190<sup>TM</sup>, POLYFLUO 200<sup>TM</sup>, POLYSILK 19<sup>TM</sup>, POLYSILK 14<sup>TM</sup> available from Micro Powder Inc., mixed fluorinated, amide waxes, for example MICROSPERSION 19<sup>TM</sup> also available from Micro Powder Inc., imides, esters, quaternary amines, carboxylic acids or acrylic polymer emulsion, for example JONCRYL 74<sup>TM</sup>, 89<sup>TM</sup>, 130<sup>TM</sup>, 537<sup>TM</sup>, and 538<sup>TM</sup>, all available from SC Johnson Wax, and chlorinated polypropylenes and polyethylenes available from Allied Chemical and Petrolite Corporation and SC Johnson wax. Mixtures and combinations of the foregoing waxes may also be used in embodiments. Waxes may be included as, for example, fuser roll release agents.

## Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. Nos. 5,290,654 and 5,302,486, the disclosures of each of which are hereby incorporated by reference in their entirety. In embodiments, toner compositions and toner particles may be prepared by aggregation and coalescence processes in which small-size resin particles are aggregated to the appropriate toner particle size, sometimes referred to herein as larger aggregates, and then coalesced to achieve the final toner particle shape and morphology.

In embodiments, toner compositions may be prepared by emulsion-aggregation processes, such as a process that includes aggregating a mixture of an optional colorant, an optional wax and any other desired or required additives, and emulsions including the resins described above, in embodiments aqueous emulsions optionally in surfactants as described above, and then coalescing the aggregate mixture. A mixture may be prepared by adding a colorant and optionally a wax or other materials, which may also be optionally in a dispersion(s) including a surfactant, to the emulsion, which may be a mixture of two or more emulsions containing the resin. The pH of the resulting mixture may be adjusted by an

## 12

acid such as, for example, acetic acid, nitric acid or the like. In embodiments, the pH of the mixture may be adjusted to from about 4 to about 5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1% to about 8% by weight, in embodiments from about 0.2% to about 5% by weight, in other embodiments from about 0.5% to about 5% by weight, of the resin in the mixture. This provides a sufficient amount of agent for aggregation.

In order to control aggregation and the subsequent coalescence of the particles, in embodiments the aggregating agent may be metered into the mixture over time. For example, the agent may be metered into the mixture over a period of from about 5 to about 240 minutes, in embodiments from about 30 to about 200 minutes, although more or less time may be used as desired or required. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 40° C. to about 100° C., and holding the mixture at this temperature for a time from about 0.5 hours to about 6 hours, in embodiments from about 1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition of the aggregation agent may be accomplished under any suitable conditions. For example, the growth and shaping

may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments from about 45° C. to about 80° C., which may be below the glass transition temperature of the resin as discussed above.

Once the desired final size of the toner particles is achieved, the pH of the mixture may be adjusted with a base to a value of from about 3 to about 10, and in embodiments from about 5 to about 9. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylenediaminetetraacetic acid (EDTA) may be added to help adjust the pH to the desired values noted above.

#### Shell Resin

In embodiments, after aggregation, but prior to coalescence, a resin coating may be applied to the aggregated particles, which forms a shell over the aggregated particles. In embodiments, a resin utilized for forming the coating and subsequent shell may be partially crosslinked in situ to form, what may be referred to, in embodiments, as a "partially crosslinked polyester resin" or a "polyester gel".

In embodiments wherein the shell is at least partially crosslinked, resins which may be partially crosslinked to form a polyester gel as a shell include, but are not limited to, the amorphous resins described above for use as the core. A single polyester resin crosslinked may be utilized to form the shell or, in embodiments, a first polyester resin may be combined with other resins to form a shell. For example, in embodiments, an amorphous resin may be combined with additional amorphous resins to form a polyester gel coating and subsequent shell. Multiple resins may be utilized in any suitable amounts. In embodiments, a first amorphous polyester resin, for example an amorphous resin of formula I above, may be present in an amount of from about 20 percent by weight to about 100 percent by weight of the total shell resin, in embodiments from about 30 percent by weight to about 90 percent by weight of the total shell resin. Thus, in embodiments, a second resin may be present in the shell resin in an amount of from about 0 percent by weight to about 80 percent by weight of the total shell resin, in embodiments from about 10 percent by weight to about 70 percent by weight of the shell resin.

In order to partially crosslink the amorphous polyester applied as a resin coating during shell formation and form a polyester gel, in embodiments it may be desirable to add a water soluble initiator to the resin utilized to form the coating to enhance crosslinking and the resulting formation of the polyester gel as a shell. Suitable water soluble initiators which may be utilized to crosslink the resin in the shell include, but are not limited to, persulfates, including potassium persulfate, ammonium persulfate, sodium persulfate, water soluble azo initiator including 2,2'-azobis[2-(2-imidazolin-2-yl)propane]dihydrochloride, 2,2'-azobis[2-(2-imidazolin-2-yl)propane]disulfate dehydrate, 2,2'-azobis(2-methylpropionamide)dihydrochloride, 2,2'-azobis[N-(2-carboxyethyl)-2-methylpropionamide]hydrate, 2,2'-azobis{2-[1-(2-hydroxyethyl)-2-imidazolin-2-yl]propane}dihydrochloride, 2,2'-azobis[2-(2-imidazolin-2-yl)propane], 2,2'-azobis(1-imino-1-pyrrolidino-2-ethylpropane)dihydrochloride, 2,2'-azobis {2-methyl-N-[1,1-bis(hydroxymethyl)-2-hydroxyethyl]propionamide}, 2,2'-

azobis[2-methyl-N-(2-hydroxyethyl)propionamide], combinations thereof, and the like.

In embodiments, water soluble initiators may be dissolved in water or a similar solvent and added to the toner reaction slurry possessing the aggregated particles. The partial crosslinking of the resin utilized to form the shell may occur while heating the slurry to a temperature of from about 25° C. to about 99° C., in embodiments from about 40° C. to about 90° C. Partial crosslinking forming the shell may take place for a period of time of from about 1 minute to about 10 hours, in embodiments from about 5 minutes to about 5 hours. In other embodiments, the crosslinking of the resin may occur during coalescence, as described below. In yet other embodiments, the resin in the shell may be partially crosslinked at the time of addition of the resin coating, with additional crosslinking of the resin coating forming the shell occurring during coalescence. In such a case, partially crosslinked at the time of addition may mean that from about 1% of the polyester to about 99% of the polyester in the shell is crosslinked at the time of addition, while from about 0% of the polyester to about 99% of the polyester in the shell is crosslinked after coalescence. In yet other embodiments, crosslinking may occur after coalescence.

The amount of initiator utilized to crosslink the polyester may be from about 0.05 percent by weight to about 20 percent by weight of the resin utilized to form the shell, in embodiments from about 0.1 percent by weight to about 10 percent by weight of the resin utilized to form the shell.

The shell resin may be applied as a coating to the aggregated particles by any method within the purview of those skilled in the art. In embodiments, the shell resin and water soluble initiator may be in an emulsion including any surfactant described above. The water soluble initiator may, in embodiments, be dissolved in water and added to the resin utilized to form the coating and subsequent shell, optionally in a slurry including any surfactant described above as suitable for forming a resin. The aggregated particles described above may be combined with said emulsion so that the polyester resin crosslinks in the presence of the water soluble initiator and forms a shell over the formed aggregates.

#### Coalescence

Following aggregation to the desired particle size and addition of the components of the shell resin with the water soluble initiators described above, which may be optionally crosslinked or partially crosslinked prior to coalescence, the particles may then be coalesced to the desired final shape, with additional crosslinking in some embodiments, resulting in crosslinked particles. Coalescence being achieved by, for example, heating the mixture to a temperature of from about 45° C. to about 100° C., in embodiments from about 55° C. to about 99° C. and/or increasing the stirring, for example to from about 400 rpm to about 1,000 rpm, in embodiments from about 500 rpm to about 800 rpm. Coalescence may be accomplished over a period of from about 1 minute to about 10 hours, in embodiments from about 5 minutes to about 5 hours. Higher or lower temperatures may be used, it being understood that the temperature is a function of the resins used for the binder.

For example, it may be desirable, in embodiments, to allow the crosslinking reaction forming the shell, or crosslinking of resins in the core, or both, to occur prior to coalescence at a temperature near the temperature utilized for coalescence of the toner particles. In other embodiments, the crosslinking reaction of the resin in the core, the shell, or both, may occur either wholly or partly during coalescence at the temperatures and times described above for coalescence. In embodiments, the reaction conditions for forming the shell may be adjusted

## 15

depending on the components utilized to form the shell. Thus, during the toner coalescence step, additional crosslinking of an unsaturated polyester resin (where crosslinking commenced prior to coalescence), in embodiments an amorphous polyester of formula I above, may be adjusted by altering the temperature and time of reaction. For example, a water soluble initiator such as ammonium persulfate may have a half life ( $t_{1/2}$ ) of about 10 hours at about 80° C., while potassium persulfate may have a half life of about 10 hours at about 60° C. Thus, in some embodiments, a lower temperature may be utilized with a water soluble initiator such as potassium persulfate, or a higher temperature may be utilized with a water soluble initiator such as ammonium persulfate.

In other embodiments, crosslinking of the amorphous resin in the core, the shell, or both, may occur after coalescence by heating the particles to a temperature of from about 70° C. to about 100° C., in embodiments from about 75° C. to about 95° C. The resulting crosslinked particles, which may be suitable for use as toner particles, thus include the reaction products obtained by contacting the amorphous resin with the water soluble initiator, including a crosslinked amorphous resin.

Crosslinking resins in the core, the resin coating used to form a shell, or both, may, in embodiments, occur while coalescing the larger aggregates within the resin coating to form a plurality of crosslinked particles possessing a core and a shell.

After aggregation and/or coalescence, the mixture may be cooled to room temperature, such as from about 20° C. to about 25° C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

Toner particles having a shell of the present disclosure may have a glass transition temperature of from about 30° C. to about 80° C. in embodiments from about 35° C. to about 70° C.

As the polyester resin utilized to form the shell has crosslinked and formed a gel the shell resin may be able to prevent any crystalline resin in the core from migrating to the toner surface. Moreover, toners of the present disclosure having partially crosslinked polyester resins in the shell may exhibit reduced peak glass in embodiments from about 20 Gardner gloss units (ggu) to about 100 ggu, in other embodiments from about 10 ggu to about 80 ggu, which may be desirable for reproduction of text and images, as some users object to high gloss and the differential which may occur between low gloss and high gloss.

## Additives

In embodiments, the toner particles may also contain other optional additives, as desired or required. For example, the toner may include positive or negative charge control agents, for example in an amount of from about 0.1 to about 10 percent by weight of the toner, in embodiments from about 1 to about 3 percent by weight of the toner. Examples of suitable charge control agents include quarternary ammonium compounds inclusive of alkyl pyridinium halides; alkyl pyridinium compounds, including those disclosed in U.S. Pat. No. 4,298,672, the disclosure of which is hereby incorporated by reference in its entirety; organic sulfate and sulfonate compositions, including those disclosed in U.S. Pat. No. 4,338,390, the disclosure of which is hereby incorporated by reference in its entirety; cetyl pyridinium tetrafluoroborates; distearyl dimethyl ammonium methyl sulfate; aluminum salts such as BONTRON E84™ or E88™ (Hodogaya Chemical); combinations thereof and the like. Such charge control agents

## 16

may be applied simultaneously with the shell resin described above or after application of the shell resin.

There can also be blended with the toner particles external additive particles including flow aid additives, which additives may be present on the surface of the toner particles. Examples of these additives include metal oxides such as titanium oxide, silicon oxide, tin oxide, mixtures thereof, and the like; colloidal and amorphous silicas, such as AEROSIL®, metal salts and metal salts of fatty acids inclusive of 10 zinc stearate, aluminum oxides, cerium oxides, and mixtures thereof. Each of these external additives may be present in an amount of from about 0.1 percent by weight to about 5 percent by weight of the toner, in embodiments of from about 0.25 percent by weight to about 3 percent by weight of the toner. Suitable additives include those disclosed in U.S. Pat. Nos. 3,590,000, 3,800,588, and 6,214,507, the disclosures of each of which are hereby incorporated by reference in their entirety. Again, these additives may be applied simultaneously with the shell resin described above or after application of the shell resin.

In embodiments, toners of the present disclosure may be utilized as ultra low melt (ULM) toners. In embodiments, the dry toner particles having a shell of the present disclosure may, exclusive of external surface additives, have the following characteristics:

(1) Volume average diameter (also referred to as "volume average particle diameter") of from about 3 to about 25  $\mu\text{m}$ , in embodiments from about 4 to about 15  $\mu\text{m}$ , in other embodiments from about 5 to about 12  $\mu\text{m}$ .

(2) Number Average Geometric Size Distribution (GSDn) and/or Volume Average Geometric Size Distribution (GSDv) of from about 1.05 to about 1.55, in embodiments from about 0.1 to about 1.4.

(3) Circularity of from about 0.9 to about 1, in embodiments from about 0.93 to about 0.98 (measured with, for example, a Sysmex FPIA 2100 analyzer).

The characteristics of the toner particles may be determined by any suitable technique and apparatus. Volume average particle diameter  $D_{50\text{v}}$ , GSDv, and GSDn may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3.

Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH. Toners of the present disclosure may possess a parent toner charge per mass ratio (Q/M) of from about  $-3 \mu\text{C/g}$  to about  $-35 \mu\text{C/g}$ , in embodiments from about  $-4 \mu\text{C/g}$  to about  $-30 \mu\text{C/g}$ , and a final triboelectric charge after surface additive blending of from  $-5 \mu\text{C/g}$  to about  $-50 \mu\text{C/g}$ , in embodiments from about  $-15 \mu\text{C/g}$  to about  $-40 \mu\text{C/g}$ .

In accordance with the present disclosure, the charging of the toner particles may be enhanced, so less surface additives may be required, and the final toner charging may thus be higher to meet machine charging requirements.

## Developers

The toner particles may be formulated into a developer composition. The toner particles may be mixed with carrier particles to achieve a two-component developer composition. The toner concentration in the developer may be from about

17

1% to about 25% by weight of the total weight of the developer in embodiments from about 2% to about 15% by weight of the total weight of the developer.

Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidene-fluoride, available, for example, as KYNAR 301<sup>TM</sup>, and/or polymethylmethacrylate, for example having a weight average molecular weight of about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu\text{m}$  in size. In embodiments from about 50 to about 75  $\mu\text{m}$  in size, coated with about 0.5% to about 10% by weight, in embodiments from about 0.7% to about 5% by weight, of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner

18

composition. However, different toner and carrier percentages may be used to achieve a developer composition with desired characteristics.

Imaging

5 The toners can be utilized for electrostatographic or xerographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengerless development (HSD), and the like. These and similar development systems are within the purview of those skilled in the art.

15 Imaging processes include, for example, preparing an image with a xerographic device including a charging component, an imaging component, a photoconductive component, a developing component, a transfer component, and a fusing component. In embodiments, the development component may include a developer prepared by mixing a carrier with a toner composition described herein. The xerographic device may include a high speed printer, a black and white high speed printer, a color printer, and the like.

20 Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser roll member. Fuser roll members are contact fusing devices that are within the purview of those skilled in the art, in which heat and pressure from the roll may be used to fuse the toner to the image-receiving medium. In embodiments, the fuser member 25 may be heated to a temperature above the fusing temperature of the toner, for example to temperatures of from about 70° C. to about 160° C., in embodiments from about 80° C. to about 150° C., in other embodiments from about 90° C. to about 140° C., after or during melting onto the image receiving substrate.

30 In embodiments where the toner resin is crosslinkable, such crosslinking may be accomplished in any suitable manner. For example, the toner resin may be crosslinked during fusing of the toner to the substrate where the toner resin is crosslinkable at the fusing temperature. Crosslinking also 35 may be effected by heating the fused image to a temperature at which the toner resin will be crosslinked, for example in a post-fusing operation. In embodiments, crosslinking may be effected at temperatures of from about 160° C. or less, in embodiments from about 70° C. to about 160° C., in other embodiments from about 80° C. to about 140° C.

40 The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 25° C.

60 EXAMPLES

Comparative Example 1

65 About 397.99 grams of a linear amorphous resin in an emulsion (about 17.03 weight % resin) was added to a 2 liter beaker. The linear amorphous resin was of the following formula:



wherein m may be from about 5 to about 1000 and was produced following the procedures described in U.S. Pat. No. 6,063,827, the disclosure of which is hereby incorporated by reference in its entirety.

About 74.27 grams of an unsaturated crystalline polyester ("UCPE") resin composed of ethylene glycol and a mixture of dodecanedioic acid and fumaric acid co-monomers with the following formula:



wherein b is from 5 to 2000 and d is from 5 to 2000 in an emulsion (about 19.98 weight % resin), synthesized following the procedures described in U.S. Patent Application Publication No. 2006/0222991, the disclosure of which is hereby incorporated by reference in its entirety, and about 29.24 grams of a cyan pigment, Pigment Blue 15:3, (about 17 weight %) was added to the beaker. About 36 grams of  $\text{Al}_2(\text{SO}_4)_3$  (about 1 weight %) was added as a flocculent under homogenization by mixing the mixture at about 3000 to 4000 rpm.

The mixture was subsequently transferred to a 2 liter Buchi reactor, and heated to about 45° C. for aggregation and mixed at a speed of about 750 rpm. The particle size was monitored with a Coulter Counter until the size of the particles reached an average volume particle size of about 6.83  $\mu\text{m}$  with a Geometric Size Distribution ("GSD") of about 1.21. About 198.29 grams of the above emulsion with the resin of formula I was then added to the particles to form a shell thereover, resulting in particles possessing a core/shell structure with an average particle size of about 8.33  $\mu\text{m}$ , and a GSD of about 1.21.

Thereafter, the pH of the reaction slurry was increased to about 6.7 by adding NaOH followed by the addition of about 0.45 pph EDTA (based on dry toner) to freeze, that is stop, the toner growth. After stopping the toner growth, the reaction mixture was heated to about 69° C. and kept at that temperature for about 1 hour for coalescence. The resulting toner particles had a final average volume particle size of about 8.07, a GSD of about 1.22, and a circularity of about 0.976.

The toner slurry was then cooled to room temperature, separated by sieving (utilizing a 25  $\mu\text{m}$  sieve) and filtered, followed by washing and freeze drying.

#### Example 1

About 398.46 grams of the linear amorphous resin of formula I from Comparative Example 1 above in an emulsion (about 17.01 weight % resin) was added to a 2 liter beaker.

15 About 82.9 grams of the unsaturated CPE resin of formula II from Comparative Example 1 above in an emulsion (about 17.9 weight % resin), and about 29.24 grams of cyan pigment, Pigment Blue 15:3, (about 17 weight %) were added to the beaker. About 35.84 grams  $\text{Al}_2(\text{SO}_4)_3$  (about 1 weight %) was added as a flocculent under homogenization by mixing the mixture at about 3000 to about 4000 rpm.

20 The mixture was subsequently transferred to a 2 liter Buchi reactor, and heated to about 45° C., for aggregation with mixing at about 750 rpm. The particle size was monitored with a Coulter Counter until the size of the particles reached an average volume particle size of about 6.97  $\mu\text{m}$  with a GSD of about 1.22.

25 A mixture of about 198.52 grams of the linear amorphous resin of formula I from Comparative Example 1 above in an emulsion (about 17.01 weight % resin) with about 3.36 grams potassium persulfate was then added to the particles at about 44.4° C. to form a shell, followed by heating to about 50.3° C. over about 2 hours, with the resulting core/shell particles having an average particle size of about 8.77  $\mu\text{m}$ , GSD 1.21.

30 Thereafter, the pH of the reaction slurry was increased to about 6.3 by the addition of NaOH followed by the addition of about 0.45 pph EDTA (based on dry toner) to freeze, that is stop, the toner growth. After stopping the toner growth, the reaction mixture was heated to about 69° C. and the pH of the reaction slurry was reduced to about 6.2 using a 0.3M  $\text{HNO}_3$  solution. The slurry was then heated to about 90° C. for about 40 2 hours to ensure crosslinking had occurred. The pH of the reaction slurry was maintained from about 6 to about 6.3 by the addition of the NaOH solution.

35 The resulting toner had a particle size of about 8.41, a GSDv of about 1.25, and a circularity of about 0.98. The toner slurry was then cooled to room temperature, separated by sieving (utilizing a 25  $\mu\text{m}$  sieve) and filtered, followed by washing and freeze drying.

40 The rheology of the toner produced was determined utilizing a dynamic temperature step method with a Dynamic Stress Rheometer SR 5000 (commercially available from Maple instrument Inc.).

45 Print gloss (Gardner gloss units or "ggu") was measured using a 75° BYK Gardner gloss meter for toner images that had been fused at a fuser roll temperature range of about 120° C. to about 210° C. (sample gloss was dependent on the toner, the toner mass per unit area, the paper substrate, the fuser roll, and fuser roll temperature).

50 As can be seen in FIG. 1, rheology measurements comparing the control toner and the toner of the present disclosure clearly demonstrate that crosslinking of the shell resin occurred during the toner preparation process of Example 1, which included the presence of the water soluble initiator. As can be seen in FIG. 2, the gloss curves demonstrate that gloss was dramatically reduced by in-situ crosslinking of the toner shell during the toner preparation process of Example 1, utilizing a water soluble initiator, as compared with the control toner.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A process for forming a toner composition comprising:
  - contacting at least one amorphous resin with at least one crystalline resin in an aqueous emulsion to form small particles, wherein the emulsion includes an optional colorant, a surfactant, and an optional wax, wherein the surfactant is present at about 0.75% to about 4% by weight of the toner composition;
  - aggregating the small particles to form a plurality of larger aggregates;
  - contacting the larger aggregates with an emulsion comprising the at least one amorphous resin or a different at least one amorphous resin, or both, to form a resin coating over the larger aggregates;
  - coalescing the larger aggregates within the resin coating and simultaneously or subsequently crosslinking either the larger aggregates or the resin coating or both, to form a plurality of crosslinked toner particles comprising a core and a shell;
  - adding at least one water soluble initiator at any stage in the process prior to the formation of the crosslinked toner particles, and
  - recovering the crosslinked toner particles.

2. The process according to claim 1, wherein the at least one amorphous resin in the small particles is the same or different as the at least one amorphous resin in the coating, and the at least one amorphous resin in the coating comprises an unsaturated polyester resin.

3. The process according to claim 1, wherein adding the at least one water soluble initiator occurs at a temperature of from about 25° C. to about 99° C. for a period of time of from about 1 minute to about 10 hours, and wherein coalescing occurs at a temperature of from about 45° C. to about 100° C., for a period of time of from about 1 minute to about 10 hours.

4. The process according to claim 1, wherein the amorphous resin is selected from the group consisting of poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, and wherein the amorphous resin of the small particles and the amorphous resin of the shell may be the same or different.

5. The process according to claim 1, wherein the at least one crystalline resin comprises a polyester selected from the group consisting of poly(ethylene-adipate), poly(propylene-adipate), poly(butylene-adipate), poly(pentylene-adipate), poly(hexylene-adipate), poly(octylene-adipate), poly(ethyl-

## 23

distearate, diglyceryl distearate, triglyceryl tetrastearate, sorbitan monostearate, cholestryl stearate, and combinations thereof, present in an amount from about 1 weight percent to about 25 weight percent of the toner particles.

8. The process according to claim 1, wherein the crosslinked toner particles have a volume average diameter of from about 3  $\mu\text{m}$  to about 25  $\mu\text{m}$ , and possess a gloss of from about 20 ggu to about 100 ggu.

9. A process for forming a toner composition comprising: contacting at least one amorphous resin with at least one

crystalline resin in an aqueous emulsion optionally in combination with at least one water soluble initiator selected from the group consisting of potassium persulfate, ammonium persulfate, sodium persulfate, 2,2'-azobis[2-(2-imidazolin-2-yl)propane]dihydrochloride, 2,2'-azobis[2-(2-imidazolin-2-yl)propane]disulfate dehydrate, 2,2'-azobis(2-methylpropionamidine)dihydrochloride, 2,2'-azobis[N-(2-carboxyethyl)-2-methylpropionamidine]hydrate, 2,2'-azobis{2-[1-(2-hydroxyethyl)-2-imidazolin-2-yl]propane}dihydrochloride, 2,2'-azobis[2-(2-imidazolin-2-yl)propane], 2,2'-azobis(1-imino-1-pyrrolidino-2-ethylpropane)dihydrochloride, 2,2'-azobis(2-methyl-N-[1,1-bis(hydroxymethyl)-2-hydroxyethyl]propionamide), 2,2'-azobis[2-methyl-N-(2-hydroxyethyl)propionamide], and combinations thereof for forming a crosslinked resin;

contacting the aqueous emulsion with an optional colorant, at least one surfactant, and an optional wax to form small particles, wherein the surfactant is present at about 0.75% to about 4% by weight of the toner composition; aggregating the small particles to form a plurality of larger aggregates;

contacting the larger aggregates with an emulsion comprising at least one amorphous resin optionally in combination with at least one water soluble initiator selected from the group consisting of potassium persulfate, ammonium persulfate, sodium persulfate, 2,2'-azobis[2-(2-imidazolin-2-yl)propane]dihydrochloride, 2,2'-azobis

## 24

bis[2-(2-imidazolin-2-yl)propane]disulfate dehydrate, 2,2'-azobis(2-methylpropionamidine)dihydrochloride, 2,2'-azobis[N-(2-carboxyethyl)-2-methylpropionamidine]hydrate, 2,2'-azobis{2-[1-(2-hydroxyethyl)-2-imidazolin-2-yl]propane}dihydrochloride, 2,2'-azobis[2-(2-imidazolin-2-yl)propane], 2,2'-azobis(1-imino-1-pyrrolidino-2-ethylpropane)dihydrochloride, 2,2'-azobis(2-methyl-N-[1,1-bis(hydroxymethyl)-2-hydroxyethyl]propionamide), 2,2'-azobis[2-methyl-N-(2-hydroxyethyl)propionamide], and combinations thereof for forming a crosslinked resin coating over the larger aggregates;

coalescing the larger aggregates possessing the resin coating to form toner particles;

heating the toner particles to a temperature of from about 70° C. to about 100° C. to crosslink the amorphous resin; and

recovering the toner particles.

10. The process according to claim 9, wherein at least one of the amorphous resin in the small particles, the amorphous resin in the resin coating, and the crystalline resin, comprises an unsaturated polyester resin.

11. The process according to claim 9, wherein the at least one water soluble initiator is added at a temperature of from about 25° C. to about 99° C., for a period of time of from about 1 minute to about 10 hours, and wherein coalescing occurs at a temperature of from about 45° C. to about 100° C., for a period of time of from about 1 minute to about 10 hours.

12. The process according to claim 9, wherein the at least one water soluble initiator is present in an amount of from about 0.05 percent by weight to about 20 percent by weight of the resin.

13. The process according to claim 9, wherein the toner particles are of a size of from about 3  $\mu\text{m}$  to about 25  $\mu\text{m}$ , possess a triboelectric charge after surface additive blending of from about  $-5 \mu\text{C/g}$  to about  $-50 \mu\text{C/g}$ , and possess a gloss of from about 20 ggu to about 100 ggu.

\* \* \* \* \*